

Sept. 25, 1956

O. E. CULLEN

2,764,515

METHOD OF SPHEROIDIZING STEEL STOCK

Filed July 22, 1954

Iron-Carbon Thermal Critical Points



Percent Carbon

Fig. 1



Fig. 2

INVENTOR.  
Orville E. Cullen  
BY  
Charles I. Haughey  
ATTORNEY

1

2,764,515

**METHOD OF SPHEROIDIZING STEEL STOCK**

Orville E. Cullen, Toledo, Ohio, assignor to Surface Combustion Corporation, Toledo, Ohio, a corporation of Ohio

Application July 22, 1954, Serial No. 445,016

7 Claims. (Cl. 148—21.5)

This invention relates to spheroidizing steel stock, and more particularly, to a comparatively rapid method for spheroidizing cementitious portions of steel stock.

In many instances, for example where severe forming operations must be performed on steel stock, either carbon steel or alloy steel, it is necessary to spheroidize the cementitious portions thereof. Spheroidization has heretofore been achieved either by extremely long heating cycles where the work is first heated to a temperature within the austenitizing range and then cooled slowly, or else cooled to about room temperature, either by quenching or by slow cooling, and then reheated to a temperature just below its  $A_{c1}$  temperature, or the minimum temperature at which, upon heating, austenite is formed. In the former method, extremely long heating cycles are required, for example 80 to 170 hours (depending on the size of the load and on the degree of spheroidization required) in the case of A. I. S. I. 1030 steel, which is known to be hard to spheroidize. The latter process is not generally used unless spheroidization is to be carried out at an intermediate processing point, since it involves a double heating operation, and it is generally equally long.

The present invention is based upon the discovery that, by proper control of processing temperatures, spheroidization can be accomplished in a fraction of the time required by former techniques.

It is therefore, an object of the invention to provide an improved spheroidizing process.

Other objects and advantages will be apparent from the description which follows, reference being had to the attached drawing, of which Fig. 1 is a portion of the iron-carbon diagram showing thermal critical points as a function of carbon content, and Fig. 2 is a typical time-temperature curve according to this invention.

According to the invention an improvement is provided in a method for spheroidizing cementitious portions of steel stock which comprises substantially austenitizing the stock by heating to a temperature at which substantially all cementite therein is converted to austenite, and cooling the stock from such temperature to a temperature substantially below the  $A_{r1}$  temperature for the stock. The improvement of the invention consists in cooling the austenitized stock to a temperature below the  $A_{r1}$  temperature for that stock, but above about 1000° F. and preferably not more than about 50° F. below the  $A_{r1}$  temperature for a time sufficiently long that a part of the austenite is converted to cementite nuclei, reheating the stock to a temperature between its  $A_{c1}$  temperature and a temperature not more than about 10° F. below its  $A_{c1}$  temperature and preferably above its  $A_{c1}$  temperature maintaining the stock at a spheroidizing temperature within the last-indicated range for a time sufficient to form spheroidized cementite, and cooling the stock. A substantially completely spheroidized microstructure is usually achieved by virtue of the above process after from about four to about ten hours at the spheroidizing temperature.

2

As a first step in spheroidizing steel according to the improved method of the invention it is necessary to heat the stock to a temperature at which cementitious portions thereof are substantially converted to austenite.

5 In the case of a hypoeutectoid steel this can be accomplished by heating above the  $A_{c1}$  temperature, or to a point at which ferrite and austenite coexist, or by carrying the heating to a higher temperature where only austenite is the stable form. In the former instance little 10 if any change in position of cementite occurs, so that spheroidized cementite appears in the finished stock in larger areas, but in approximately the same positions that the cementite deposits, in another form, were present in the original stock. In the latter case, substantially the 15 entire stock becomes austenitic so that a redistribution of cementitious portions, after spheroidizing occurs. In the instance of hypereutectoid steel, complete austenitizing occurs only upon heating above the  $A_{cm}$  temperature, which is a function of carbon content. In practice 20 it is often preferred to austenitize at temperatures somewhat below the  $A_{cm}$  line, but sufficiently high to austenitize substantially all the cementite. Since only austenite is the stable form at austenitizing temperatures above 25 the  $A_{cm}$  line for hypereutectoid steel, it will be apparent that substantial migration of carbon, or  $Fe_3C$ , and therefore of the location of spheroidized particles in the finished product, can be expected in this type of steel. The preferred range of austenitizing temperatures as a function of carbon content is represented for unalloyed, or 30 carbon steel, by the shaded portion of the attached drawing.

As is above stated, in practicing the method of the invention, the austenitized stock is cooled to a temperature below its  $A_{r1}$  temperature, but not lower than about 35 1000° F., as a second step. Although the invention is not limited to the following theoretical explanation, it is believed that, upon cooling to a temperature within the indicated range, cementite nuclei are precipitated from the stock and, upon subsequent reheating at a temperature near the  $A_{c1}$  temperature, additional cementite precipitated from the austenitic phase forms spherules around these nuclei. In this connection it has been observed that maintaining the stock below the  $A_{r1}$  temperature for a longer period of time tends to produce smaller 40 spherules than does maintaining the stock at such temperature for a relatively short period of time. This difference is believed to be attributable to the formation, in the former instance, of a larger number of nuclei around which the spherules form, as compared with a smaller 45 number of nuclei around which larger spherules form in the latter instance. It has also been observed that cementite precipitation which occurs during this step of the method of the invention should be terminated, by reheating as hereinafter described in more detail, before 50 the stock is converted to a relatively stabilized pearlitic form. If the precipitation of cementite is allowed to proceed, during this stage, until the stock contains substantial amounts of pearlite, it is found that subsequent spheroidization proceeds only with substantial difficulty and at a relatively low rate. It is preferred that this cementite precipitation step of the method of the invention be terminated before substantial equilibrium is reached, or while some austenite remains in the stock. It is also preferred that the stock be quenched from the austenitizing 55 temperature, or at least from between the  $A_{c1}$  and the  $A_{r1}$  temperatures after austenitizing, to the temperature at which cementite is precipitated, as described, because the process can be substantially speeded-up by virtue of such quenching since the time required for such cooling is essentially lost time, and since precipitation occurs more rapidly at comparatively low temperatures. However, as 60 hereinafter described in more detail, the entire spher- 65 70 75 80 85 90 95

odizing process according to the invention can be carried out in a single continuous furnace, if desired.

The final step in spheroidizing steel stock according to the invention is reheating to a temperature between its  $Ac_1$  temperature and a temperature not more than about 10° F. below its  $Ar_1$  temperature and preferably above its  $Ar_1$  temperature, and maintaining the stock within such range for from about four hours to about ten hours. When the stock has been cooled, prior to this reheating, as described in the preceding paragraph, spheroidization proceeds rapidly at temperatures within such range, with the result that even hard to spheroidize stock is substantially completely spheroidized within the indicated time.

The attached drawing shows one specific iron-carbon diagram whereon the differences between the various critical points upon heating and cooling are represented. It is known that differences between these critical points are a function of the composition of the particular metal being studied. In consequence, in order to illustrate the various critical temperatures of all alloy steels, or even for all grades of carbon steels, it would be necessary to prepare a separate diagram for each such steel. However, it is generally true that the  $A_1$  change, which term is used herein and in the appended claims in its usual and accepted sense, namely to indicate the minimum temperature at which austenite forms or disappears as a stable constituent of a steel, occurs at a higher temperature upon heating ( $Ac_1$ ) than upon cooling ( $Ar_1$ ), for any given steel. A detailed discussion of the thermal critical points for steel will be found in *The Metallography and Heat Treatment of Iron and Steel*, pages 110-128 of the 1926 edition, Albert Sauveur. The specific temperatures shown on the attached drawing must be considered as exemplary only, however, because of the differences in these specific temperatures which occur with differences in composition.

If the particular temperatures, especially the  $Ac_1$  and the  $Ar_1$  temperatures, of a particular stock which it is desired to spheroidize according to the invention are not known, they can readily be determined according to procedures described in the Sauveur reference, cited above. In many cases, however, the temperatures can be approximated with sufficient accuracy from the attached drawing.

The following example is presented solely for the purpose of further illustrating and disclosing the invention, and is in no way to be considered as a limitation thereon.

#### Example

Samples of A. I. S. I. 1030 steel were continuously spheroidized in a furnace schematically illustrated on the last page of a reprint entitled "Continuous Short-Cycle Anneals for Spheroidization of Cartridge-Case Steel," originally published in *Metal Progress*, July 1953. The  $Ac_1$  temperature of this stock was about 1340° F., while the  $Ar_1$  temperature was about 1250° F. The furnace controllers were set so that the stock was heated to about 1380° F. in approximately 3 1/4 hours in an initial heating zone, maintained at about 1380° F. for approximately two hours in an austenitizing zone, cooled to about 1245° F. in about 1 1/2 hours and maintained at about 1245° F. for approximately 3/4 hour in a nucleating zone, reheated to about 1325° F. and maintained at such temperature for approximately eight hours in a spheroidizing zone, and then cooled to about 1100° F. in approximately 2 1/4 hours in a final cooling zone. The work was then discharged from the furnace. Samples, after polishing and etching, were examined and found to show substantially completely spheroidized structures.

It is known that the displacement of the critical temperatures of steels from the theoretical equilibrium critical temperatures as currently published will vary both with the composition of the steel and the rate of heating or cooling. In Fig. 2 this has been illustrated by the curves of the converging  $Ac_1$  and  $Ar_1$  lines. The superimposed annealing cycle curve of Fig. 2 will in fact be a wavy line

due to the practical impossibility of maintaining constant furnace temperatures. It has been demonstrated that carbides, in the form of pearlite or cementite, will dissolve less readily into austenite than they precipitate therefrom, the classic demonstration of this being the carburization of steel to up to 3 1/2 or so per cent carbon at about 1700° F. in less than one hour for thin steel strips, in a carburizing atmosphere whose carbon potential is limited by phase rule considerations to the  $Ac_m$  line, or about 1.2% carbon. Considering these facts, it is apparent that on the sub-critical annealing portion of this process, the apparent  $Ac_1$  line for the steel treated in a given furnace may be higher than the text-book figures, since it is necessary only to periodically drop the work being annealed to below the  $Ac_1$  critical temperature to cause the spheroidizing to proceed. In such a case the cementite which is agglomerated as spherules below the  $Ac_1$  line as the temperature wavers therabout will not substantially redissolve into the austenite during the moments the work is actually above the theoretical  $Ac_1$  line. For this reason the illustrated  $Ac_1$  and  $Ar_1$  lines may appear too widely spaced in Fig. 2, but in fact they represent a close approach to the practical temperatures with which one must work in industrial heating equipment.

It will be apparent that the method of the invention is not limited to a spheroidizing cycle carried out in a furnace or furnaces, as salt or other liquid baths could equally well be used for carrying out the various heating operations involved therein. It will also be apparent that other changes and modifications can be made from the specific details disclosed and described without departing from the spirit of the attached claims.

I claim:

1. In a method for spheroidizing cementitious portions of steel stock which comprises austenitizing the stock by heating to a temperature at which cementite therein is converted to austenite, and cooling the stock from such temperature to a temperature below the  $Ar_1$  temperature for the stock, the improvement which consists in cooling the austenitized stock to a temperature below its  $Ar_1$  temperature, but not lower than about 1000° F. for a time sufficiently long that a part of the austenite is converted to cementite nuclei, but not sufficiently long for the formation of a relatively stable pearlitic structure, reheating the stock to a temperature between its  $Ac_1$  temperature and its  $Ar_1$  temperature, maintaining the stock at a temperature within the last-identified range for from about four hours to about ten hours, and cooling the stock, whereby a spheroidized microstructure is achieved.
2. In a method for spheroidizing cementitious portions of steel stock which comprises austenitizing the stock by heating to a temperature at which substantially all cementite therein is converted to austenite, and cooling the stock from such temperature to a temperature below the  $Ar_1$  temperature for the stock, the improvement which consists in cooling the austenitized stock to a temperature below its  $Ar_1$  temperature but above about 1000° F. for a time sufficiently long that a part of the austenite is converted to cementite nuclei, but not sufficiently long for the formation of a relatively stable pearlitic structure, reheating the stock to a temperature between its  $Ac_1$  temperature and a temperature not more than about 10° F. below its  $Ar_1$  temperature, maintaining the stock at a temperature within the last-identified range for from about four hours to about ten hours, and cooling the stock, whereby a substantially completely spheroidized microstructure is achieved.
3. In a method for spheroidizing cementitious portions of steel stock which comprises austenitizing the stock by heating to a temperature at which substantially all cementite therein is converted to austenite, and cooling the stock from such temperature to a temperature below the  $Ar_1$  temperature for the stock, the improvement which consists in cooling the austenitized stock to a temperature between the  $Ar_1$  temperature and the  $Ac_1$  tempera-

70  
75

ture, rapidly cooling the stock to a temperature below its  $Ar_1$  temperature but above about  $1000^{\circ}$  F. for a time such that only a portion of the austenite is converted to cementite nuclei, reheating the stock to a temperature between its  $Ac_1$  temperature and a temperature not more than about  $10^{\circ}$  F. below its  $Ar_1$  temperature, maintaining the stock at a temperature within the last-identified range for from about four hours to about ten hours, and cooling the stock, whereby a substantially completely spheroidized microstructure is achieved.

4. In a method for spheroidizing cementitious portions of steel stock which comprises austenitizing the stock by heating to a temperature at which cementite therein is converted to austenite, and cooling the stock from such temperature to a temperature below the  $Ar_1$  temperature for the stock, the improvement which consists in cooling the austenitized stock to a temperature below its  $Ar_1$  temperature, but not more than about  $50^{\circ}$  F. therebelow, maintaining the stock at a temperature within the last-identified range for a time sufficiently long that at least a part of the austenite is converted to cementite nuclei, reheating the stock to a temperature between its  $Ac_1$  temperature and a temperature not more than about  $10^{\circ}$  F. below its  $Ar_1$  temperature, maintaining the stock at a temperature within the last-identified range until a substantially completely spheroidized microstructure is achieved.

5. In a method for spheroidizing cementitious portions of steel stock which comprises austenitizing the stock by heating to a temperature at which cementite therein is converted to austenite, and cooling the stock from such temperature to a temperature below the  $Ar_1$  temperature for the stock, the improvement which consists in quenching the austenitized stock to a temperature below its  $Ar_1$  temperature, but above about  $1000^{\circ}$  F., maintaining the stock at a temperature within such range for a time such that a part only of the austenite is converted to cementite nuclei, reheating the stock to a temperature between its  $Ac_1$  temperature and a temperature not more than about  $10^{\circ}$  F. below its  $Ar_1$  temperature, maintaining the stock at a temperature within the last-identified range for from about four hours to about

ten hours, and cooling the stock, whereby a substantially completely spheroidized microstructure is achieved.

5 6. In a method for spheroidizing cementitious portions of steel stock which comprises austenitizing the stock by heating to a temperature at which cementite therein is converted to austenite, and cooling the stock from such temperature to a temperature below its  $Ar_1$  temperature, the improvement which consists in cooling the austenitized stock to a temperature below its  $Ar_1$  temperature, but not lower than about  $1000^{\circ}$  F. for a time sufficiently long that at least a part of the austenite is converted to cementite nuclei, reheating the stock to a temperature between its  $Ac_1$  temperature and a temperature not more than about  $10^{\circ}$  F. below its  $Ar_1$  temperature, maintaining the stock at a temperature within the last-identified range until a substantially completely spheroidized microstructure is achieved, and cooling the stock.

10 7. In a method for spheroidizing cementitious portions of steel stock which comprises austenitizing the stock by heating to a temperature at which cementite therein is converted to austenite, and cooling the stock from such temperature to a temperature below its  $Ar_1$  temperature, the improvement which consists in cooling the austenitized stock to a temperature below its  $Ar_1$  temperature, but not lower than about  $1000^{\circ}$  F. for a time sufficiently long that at least a part of the austenite is converted to cementite nuclei, but not sufficiently long for the formation of a relatively stabilized pearlitic structure, reheating the stock to a temperature between its  $Ac_1$  temperature and a temperature not more than about  $10^{\circ}$  F. below its  $Ar_1$  temperature, maintaining the stock at a temperature within the last-identified range until a substantially spheroidized microstructure is achieved, and cooling the stock.

#### References Cited in the file of this patent

#### UNITED STATES PATENTS

|           |           |               |
|-----------|-----------|---------------|
| 2,181,947 | McCarroll | Dec. 5, 1939  |
| 2,188,155 | Payson    | Jan. 23, 1940 |
| 2,368,418 | McCarroll | Jan. 30, 1945 |
| 2,376,454 | Schneider | May 22, 1945  |